

Oct. 22, 1929.

S. I. SALZMAN

1,732,244

METHOD OF HARDENING STEEL

Filed March 29, 1928



Fig. 1



Fig. 2

Fig. 3

Fig. 4

Fig. 5

Inventor  
Samuel I. Salzman

John W. Darley  
Attorney

## UNITED STATES PATENT OFFICE

SAMUEL I. SALZMAN, OF BALTIMORE, MARYLAND

## METHOD OF HARDENING STEEL

Application filed March 29, 1928. Serial No. 265,536.

My invention relates to a method of hardening steel.

The principal object of my invention is to devise a method of hardening steel which is characterized by a uniformity of product, free from internal strains and tendency to warp, and an imparting to the steel any desired degree of elasticity, toughness, and capacity for resisting shock.

10 A further object is to devise a method as above described, and particularly one that is adapted for the hardening of thin steel, which is characterized by a high production rate, with a minimum of handling on the part of 15 the operator.

A further object is to devise a method of hardening thin steel sheets in the form of razor blades which is designed to effect a substantially individual treatment of the 20 blades without preventing the attainment of a favorable rate of manufacture.

A further object is to devise an apparatus for performing the hardening or tempering steps of the method which is designed to effect 25 the chilling of the heated steel with marked rapidity, while at the same time absolutely preventing the creation of a warped condition through inadequately relieving the internal strains.

30 My improved method and the apparatus for effectuating the same are more particularly intended for use in the heat treatment of thin razor blades of a well known type. As now practiced in the art, the blade blanks, 35 after perforation and forming, are assembled in stacked and interleaved relation on a frame with sheets having a high heat conductivity, usually copper. This assembly is then clamped, subjected to heat, and finally chilled

40 to harden the blade blanks, the copper sheets serving both to conduct heat inwardly to and outwardly from the uncovered areas of the blanks.

The practice of the foregoing method prevents penetration of the blanks by oxidation, 45 except over limited areas, during the heating and chilling operations, an effect which would otherwise render the blanks useless owing to their thinness. Aside from this preventive 50 ability, the method is characterized by cer-

tain disadvantages which detract from its desirability for use. The stacking of the blades not only requires undue time and labor, but the manifest difficulty of uniformly clamping, heating, and cooling the blanks quickly at a uniform rate results in the production of blades having varying qualities and capacities for maintaining a cutting edge.

The method and apparatus embodied in the present application are intended to conserve 55 the advantage of the older type of heat treatment in respect of preventing oxidation, while at the same time substantially effecting an individual treatment of the blanks, thus satisfying the ideal requirements. Notwithstanding this advantage, the production rate 60 is not lessened, owing to the improved mode of handling, and may in reality be increased over existing methods. The product is characterized by a marked uniformity of structure, with a resulting capacity for withstand- 65 ing shock and maintaining a cutting edge over a longer period of time than now obtains in the art.

For purposes of disclosure, the method and 70 apparatus are described with reference to the manufacture above noted, but it will be obvious that application of the central idea involved may be made with equal facility to other products such as wire, springs of various types, and other articles requiring heat 75 treatment.

These and further objects of my invention will be set forth in the following specification, reference being had to the accompanying 80 drawing, and the novel means by which said objects are effectuated will be definitely pointed out in the claims.

In the drawing: 85

Fig. 1 is a diagrammatic view in side elevation showing the various apparatus utilized in carrying out my improved method, arranged in the order of their operation.

Figs. 2, 3 and 4 are sections taken along lines of the same respective numerical designation in Fig. 1, looking in the direction of the respective arrows.

Fig. 5 is a plan view of the steel strip as it is passed through the various apparatus for hardening purposes.

A steel strip 10 of any desired length and having a width and thickness appropriate for thin razor blades is first perforated to form the usual openings 11 and 12, and is scored as at 13 to indicate the end edges of the blades. These operations are performed prior to the hardening and the strip may then be fed directly to the apparatus hereinafter described, or it may be wound on a spindle 14 in the manner indicated by the numeral 15. From the spindle 14, the strip 10 is unwound and drawn through the various apparatus herein-after described by a pair of coating rollers 16, appropriately mounted and suitably driven, between which said strip passes.

The first step in my improved method is the heating of the strip 10 to a predetermined temperature which is effected by passage through a tube 17 of approved cross section which is arranged in a furnace 18 provided with a burner 19. The strip 10 is propelled by the rollers 16 at a predetermined, constant speed and the furnace 18 is of a length adequate to insure the heating of the strip 10 to the desired temperature before it issues therefrom.

Immediately adjacent the delivery opening of the tube 17 is arranged the apparatus for effecting the chilling of the heated strip for hardening the same. This apparatus comprises a pair of coating chambers 20 and 21, preferably arranged in vertical relation, with the strip 10 passing therebetween and subjected to the weight of the upper casing 20. A chilling fluid 22 passes continually through said casings, ducts 23 and 24 communicating with the upper casing 20 for this purpose and ducts 25 and 26 with the lower casing 21. Said casings are preferably formed of a material having a high heat conductivity, so that the heated strip 10 in passing therebetween will be quickly chilled, the abstracted heat being conducted to the chilling medium 22.

In order to relieve any internal strains that may be present in the strip 10 after being subjected to the action of the chilling medium and to properly temper the same for insuring the obtention of a fine cutting edge, said strip next passes between a pair of coating channel frames 27 and 28, also arranged in vertical relation, the bases of said frames serving to clamp said strip under the weight of the upper frame 27 and the up-standing sides thereof to properly confine the heat received from burners 29 and 30. During passage between said frames, the strip will be again heated, but to a temperature less than the initial temperature received in the furnace 18.

After leaving this second heated zone, the strip 10 is again chilled by moving between coating casings 31 and 32 which are similarly arranged and constructed to the casings 20 and 21. The heat treatment of the strip 10

is then completed, after which it may be severed along the scored lines 13 to form the blade blanks which may then be ground and polished in any approved manner.

It will be observed that, according to my improved method, the heat treatment is a continuous operation, thus insuring a high production rate even though the successive blade blank portions of the strip 10 are treated individually. Two desirable, but heretofore conflicting characteristics, are therefore successfully combined. Heating and chilling of the strip 10 are effected without oxidation thereof or contact with the flame or chilling medium and moreover, adequate pressure is maintained during the chilling and second heating operation to prevent warping of the strip. However, the latter pressure will not be sufficiently great to prevent movement of the strip 10 by the rolls 16 and this pressure may be exerted either in the manner shown, under the action of gravity, or it may be effected mechanically, which would permit the positioning of the chilling casings and heating frames in other positions than vertical.

The product resulting from this mode of treatment possesses a high degree of elasticity without affecting its capacity for receiving and maintaining a cutting edge over a considerable period of time, characteristics which are highly desirable in razor blades. As before stated, it is contemplated that the strip 10 will be propelled through the various steps of the process by the rollers 16 at a constant rate of speed, which mode of handling has been found suitable for the heat treatment of razor blades, but it will be obvious that other types of products might require a varying or intermittent rate of speed.

While I have shown one set of elements and combinations thereof for effecting my improved method and apparatus for the heat treatment of steel, it will be understood that the same are intended for the purpose of illustration only and in nowise to restrict the same to the exact steps and combinations shown, for many changes may be made therein without departing from the spirit of my invention.

I claim:

1. The herein described method of hardening lengths of steel which consists in drawing the same successively through a heated zone, a chilled zone, a second heated zone, and a second chilled zone to harden the original length progressively, a predetermined pressure being maintained on the portions of said steel passing through said chilled zones and said second heated zone and said steel being maintained free from contact with the chilling medium employed.

2. The herein described method of hardening lengths of thin steel which consists in passing the same successively through a

heated zone, a chilled zone, a second heated zone including the application of heat to the opposite sides of said steel, and a second chilled zone to harden and temper the original length progressively, a predetermined pressure being maintained on the portions of said steel passing through said chilled zones and said second heated zone, and said steel being maintained free from contact with the chilling medium employed.

10 In testimony whereof, I affix my signature.  
SAMUEL I. SALZMAN.

15

20

25

30

35

40

45

50

55

60

65